

# United States Patent Office

3,080,221

Patented Mar. 5, 1963

1

3,080,221

FUELS FOR INTERNAL COMBUSTION ENGINES  
 Karl Nützel, Köln-Stammheim, and Rudolf Stroh, Eugen  
 Himmens, and Walter Lohmar, Leverkusen, Germany,  
 assignors to Farbenfabriken Bayer Aktiengesellschaft,  
 Leverkusen, Germany, a corporation of Germany  
 No Drawing. Filed Jan. 24, 1961, Ser. No. 84,525  
 3 Claims. (Cl. 44—69)

The present invention relates to fuels for internal combustion engines of the spark ignition type, especially to motor fuels for cars and airplanes; more particularly it concerns motor fuels consisting of gasoline or mixtures of gasoline and benzene. According to the invention these fuels contain boron compounds of the general formula



wherein the three Ar represent the same or different aromatic radicals which are substituted by at least three aliphatic hydrocarbon radicals having 1—10 carbon atoms, two of the hydrocarbon radicals being in o,o-position to the boron atom.

Owing to the presence of boron compounds of the above general formula the tendency of the motor fuels to form deposits in the combustion engines is minimized. This applies particularly to motor fuels which contain anti-knock agents, for instance lead compounds such as lead tetraethyl, or aromatic amines such as monomethyl aniline, N-methyl-p-toluidine and xylidine or mixtures thereof. Furthermore the boron compounds improve the octane number of the fuels and prevent the progressive increase in the minimum requirements for the fuels on prolonged operation of the engines.

Suitable boron compounds of the formula indicated are for instance boron trimesityl of the formula



boron trimesityl of the formula



and boron triduryl of the formula



2

These compounds can be obtained by reacting boron trifluoride with the Grignard compounds of trimethylchloride, triisopropylphenylchloride or durylchloride in known manner.

5 The content of the boron compounds in the fuels may vary within wide limits. It may for instance amount to .001%—5% by volume. The ratios depend in the first place upon the content of the anti-knock agents in the motor fuels; suitable ratios can easily be determined by 10 preliminary tests.

The following examples serve to illustrate the invention without, however, limiting the scope thereof.

## Example 1

15 A gasoline whose physico-chemical data are indicated below was mixed with .03% by volume of lead tetraethyl and .05% by volume of boron trimesityl, boron tristriisopropylphenyl or boron triduryl. With this fuel a four cylinder motor was operated under changing load 20 for 25 hours without interruption. After this time only about 5% of the surface of the pistons were covered with a light, very thin weakly brownish coating. The pistons did not show further alterations. On the bottom 25 of the pistons and on the walls of the combustion chambers a slight coating of a white greyish powder was observed, but no hard carbonaceous deposits of combustion residues were present. In the suction system no alterations could be observed.

The physico-chemical data of the gasoline used were 30 as follows.

Density at 15° C. .... .735 g./ml.  
 Octane number (IG motor test) .... 70.7.  
 Vapour pressure (Reid) .... .55 kg./m.<sup>2</sup>.  
 Content of lead (TEL) .... .0.  
 35 Sulfur .... .06% by weight.  
 Residue test (ASTM) .... 7 mg./100 ml.

### Distillation analysis:

40 Initial boiling point .... 32° C.  
 Distillation up to 75° C. .... 23.4% by volume.  
 Distillation up to 100° C. .... 36.6% by volume.  
 Distillation up to 150° C. .... 65.8% by volume.  
 Distillation up to 200° C. .... 97.3% by volume.  
 Dry point .... 205° C.

45 When the test was carried out under equal conditions with the same gasoline and with the addition of .03% by volume of lead tetraethyl but without the addition of boron trimesityl, boron tristriisopropylphenyl or boron triduryl 22% of the surface of the pistons were covered with a lacquer-like coating and the bottom of the pistons 50 as well as the walls of the combustion chambers were covered with hard carbonaceous combustion residues.

If .05% by volume of boron triphenyl which is known as additive to motor fuels, was applied instead of the 55 boron compounds of the invention, 17% of the surface of the pistons were covered with a lacquer-like coating; besides, disturbances occurred in the carburetor on account of cloudy precipitates.

## Example 2

60 A gasoline having the same physico-chemical data as the gasoline of Example 1 but which did not contain lead tetraethyl was mixed with .5% by volume of boron trimesityl. The octane number determined by the F<sub>1</sub>-method (ASTM D908—51) in the IG-motor test amounted 65 to 71.1; with the addition of 1% by volume of boron trimesityl it amounted to 71.6 whereas without the addition of boron trimesityl the octane number was 70.7.

When instead of .5% by volume of boron trimesityl the 70 same amount of boron tristriisopropylphenyl or boron triduryl was applied the octane number was 72.7 or 72.1 respectively.

Very remarkable is the stability the boron compounds of the invention exhibit in the motor fuels. If for instance a solution of 5 g. of boron trimesityl, 5g. of boron tristriisopropylphenyl or 5 g. of boron triduryl in 60 ml. of a benzene-ligroin mixture is shaken with 40 ml. of water and kept standing at room temperature for 70 hours, no hydrolysis of the boron compounds can be observed. If however a solution of 5 g. of boron triphenyl in 60 ml. of a benzene-ligroin mixture is shaken with 40 ml. of water and kept standing at room temperature for 70 hours, 29% by weight of the boron triphenyl are hydrolysed and have become inefficient.

What we claim:

1. A motor fuel for an internal combustion engine of the spark ignition type, comprising a component selected from the group consisting of gasoline, benzene, and an admixture of gasoline and benzene, together with about .001% to 5% by volume of a boron compound having the general formula



wherein Ar represents an aromatic radical having at least three aliphatic hydrocarbon substituents having from

about 1 to 10 carbon atoms, two of said aliphatic hydrocarbon substituents being in o,o-position with respect to the boron atom.

5 2. A motor fuel according to claim 1 wherein the boron compound is selected from the group consisting of boron trimesityl, boron tristriisopropylphenyl and boron triduryl.

10 3. A motor fuel according to claim 1 containing at least one antiknock additive selected from the group consisting of lead tetraethyl, monoethyl aniline, N-methyl-p-toluidine, and xylidine.

References Cited in the file of this patent

UNITED STATES PATENTS

15 2,410,846 Walters ----- Nov. 12, 1946

FOREIGN PATENTS

549,075 Great Britain ----- Nov. 5, 1942

OTHER REFERENCES

"Boron New Improvement Agent," an article by Hughes et al. in Refining Engineering, vol. 28, No. 7, July 1956, pages C10-C13.